

## UNITED STATES PATENT OFFICE

2,639,219

NONCAKING POTASSIUM BROMIDE FOR  
PHOTOGRAPHIC DEVELOPERS

Edwin S. Wiitala and William J. Rogers, Rochester, N. Y., assignors to Eastman Kodak Company, Rochester, N. Y., a corporation of New Jersey

No Drawing. Application March 28, 1952,  
Serial No. 279,208

6 Claims. (Cl. 23—89)

1

This invention relates to the prevention of caking of potassium bromide, and more particularly to potassium bromide in which a desiccating agent which is compatible with photographic developers has been incorporated. Such agents impart non-caking properties to the potassium bromide.

Potassium bromide is an important component of most photographic developers and acts essentially as an antifogging agent. To insure good uniformity of mixing in preparing developer formulations for packaging, it is usually necessary to employ potassium bromide having a relatively fine screen analysis. Most potassium bromide is approximately 60 to 80 mesh or finer.

A great disadvantage of potassium bromide is its very severe tendency to cake upon storage. Therefore, almost invariably, before a developer mixture can be made, the supply of potassium bromide from which a component part is to be selected to be added to the developer mixture has to be broken up, granulated and screened. In fact, certain lots have been found to be so badly caked that they have been totally rejected for use.

An object of the present invention is, therefore, to provide a non-caking potassium bromide which is suitable for employment in photographic developer mixtures.

Another object of the invention is to provide a method of producing a non-caking potassium bromide.

In accordance with the invention we have discovered that the addition of small quantities of a desiccating agent, including one or more of the following boron compounds, boric anhydride ( $B_2O_3$ ), metaboric acid and orthoboric acids, have marked effect upon reducing the caking of potassium bromide. The potassium bromide and the desiccating agent may be mixed together in any suitable manner. Quantities of desiccating agent in an amount as small as  $\frac{1}{2}\%$  of the weight of potassium bromide is effective in preventing caking. We have found that such small amounts of these desiccating agents when introduced into the developer formulations have no effect upon the photographic properties of the developer. Slight changes in the alkalinity of the developer formulation produced by the presence of these boron compounds can be adjusted by a minor adjustment of the alkaline component of the mixture. While these boron compounds in an amount of  $\frac{1}{2}$  to  $1\%$  of the weight of potassium bromide to be treated is preferred, amounts up to  $10\%$  could be advantageously employed.

The invention will be further illustrated in the following examples:

2

## Example 1

The advantages of the invention can be demonstrated as follows: A sample of fine granular, 80 mesh, potassium bromide and a similar sample containing 0.05%  $B_2O_3$  were conditioned at 120° F. for a week with intermittent heating and cooling to room temperature. The untreated sample was caked and slightly discolored by this heating. The sample containing the  $B_2O_3$  addition was found to be perfectly free flowing and to be unchanged in appearance.

## Example 2

15 The procedure of Example 1 was repeated except that 1% by weight of boric anhydride was employed to overcome the caking tendency of the potassium bromide. As in the first example, the untreated sample caked but the treated sample 20 was free flowing.

## Example 3

25 The same procedure as in Example 1 was followed, except that 0.5% metaboric acid was used to overcome caking. The potassium bromide showed no tendency to cake with metaboric acid as a cake preventing agent.

## Example 4

30 The same procedure as in Example 1 was followed, except for the substitution of  $\frac{1}{2}\%$  orthoboric ( $H_3BO_3$ ) for the boric anhydride. The potassium bromide containing the orthoboric acid was free flowing, while the check sample of 35 straight potassium bromide was moderately caked.

Our invention, therefore, is a desirable contribution to the photographic developing art in that it permits saving of materials and enables 40 potassium bromide to be handled and combined with other components of the photographic developers more easily.

What we claim and desire to secure by Letters Patent of the United States is:

- 45 1. A finely divided non-caking potassium bromide composition containing as an anti-caking agent 0.05% to 10% by weight of a compound selected from the group consisting of boric anhydride, metaboric acid and orthoboric acids.
- 50 2. A finely divided non-caking potassium bromide composition containing as an anti-caking agent 0.05% to 10% by weight of boric anhydride.
- 55 3. A finely divided non-caking potassium bromide composition containing as an anti-caking agent 0.05% to 10% by weight of metaboric acid.
4. A finely divided non-caking potassium bro-

mide composition containing as an anti-caking agent 0.05% to 10% by weight of orthoboric acid.

5. The method of preventing caking of finely divided potassium bromide which comprises mixing therewith a small amount of a non-caking agent selected from the group consisting of boric anhydride, metaboric acid and orthoboric acid.

6. The method of preventing caking of finely divided potassium bromide which comprises mixing therewith  $\frac{1}{2}$  to 1% by weight of boric an- 10 hydride.

EDWIN S. WIITALA.  
WILLIAM J. ROGERS.

## References Cited in the file of this patent

## UNITED STATES PATENTS

| Number      | Name           | Date          |
|-------------|----------------|---------------|
| 5 2,313,523 | Donovan et al. | Mar. 9, 1943  |
| 2,477,323   | Wood           | July 26, 1949 |